

## UNITED STATES PATENT OFFICE

2,000,689

## WOOD STAINING

William Stansfield Calcott, Pennsgrove, and Charles J. Pedersen, Carneys Point, N. J., assignors to E. I. du Pont de Nemours & Company, Wilmington, Del., a corporation of Delaware

No Drawing. Application December 23, 1930,  
Serial No. 504,426

7 Claims. (Cl. 91—68)

This invention relates to the staining of fibrous materials and more particularly to the production of stains by the catalytic oxidation of organic compounds on said fibrous materials.

5 Heretofore wood has been stained by one or two general methods. By the first method the wood to be stained was treated with dye solutions to allow it to absorb the dyes. The great objection to the use of this method has been the poor penetration attained.

10 By the other method the staining has been accomplished by the oxidation of aromatic organic compounds on the wood fibres, the oxidation being brought about by the use of chemical oxidizing agents in the presence of mineral acids. The disadvantages of this last named method were the resultant tendering of the wood and the efflorescence of the resultant compounds on the surface of the wood.

15 This invention has for an object the production of a stain with great penetrating power and insolubility. A further object is the staining of fibrous materials without use of chemical oxidizing agents and mineral acids. Still further objects are the production of a material adapted for 20 rapid staining of wood, the production of a very fast stain, a very deep stain, a stain which is unaccompanied by tendering of the fiber, a stain which is unaccompanied by efflorescence and in general an advancement of the art. Other objects will appear hereinafter.

25 These objects are accomplished by this invention by which certain substituted amines or di-30 amines are catalytically oxidized on or in the material to be stained. The invention will be readily understood from a consideration of the following examples in which the parts are given by weight.

*Example I*

35 There was dissolved in 75 ml. of the mono-ethyl-ether of ethylene glycol 1 gm. of cupric chloride, and to the solution was added 25 ml. of toluene. Fifteen (15) gms. of m-toluylene di-40 amine was dissolved in the resultant mixture. A piece of wood was heated to the temperature of 150° F. and then dipped into the solution while still warm. The wood was allowed to soak for 30 minutes after which it was withdrawn wiped, dried and finished. In the examples carried out 45 it has been found that cooling the wood in the solution greatly aids the penetration of the stain.

*Example II*

50 In this example all figures are based upon the original weight of the alcohol. To a 1% solution

of cupric chloride in alcohol there was added sufficient aqua ammonia to form the copper-ammonia complex. The resultant solution was a clear violet and to it was added 15% of m-toluylene di-amine. The wood to be stained was allowed to remain in this solution for about 30 minutes after which it was withdrawn wiped and dried by heat. In this and in the other examples, drying at room temperature has also been found satisfactory.

*Example III*

55 A sample of wood was first soaked in a 15% solution of m-toluylene di-amine in alcohol. Thereafter the surface liquid was wiped off and the wood dipped into a 1% solution of cupric chloride in alcohol. Oxidation started immediately at the surface and although the color developed below the surface of the wood somewhat slowly due to the rate of diffusion of the air to the interior of the wood, the visible portions of the wood were stained even when scraped to the depth of the penetration of the m-toluylene di-amine.

60 Other organic compounds than the m-toluylene di-amine of the above examples may be used satisfactorily. In general other aromatic di-amines, for example, m-phenylene-di-amine, p-phenylene-di-amine, and m-naphthylene-di-amine, are suitable. There may also be used aromatic amines which are characterized by containing activating or positive groups, for example, the hydroxyl, the alkoxy and amino groups in the ring and containing no negative groups or substituents, such as, the carboxyl, the sulphonate and nitrile groups in the ring. As examples of suitable compounds of this class there may be mentioned p-amino-phenol and p-amino-anisole. As examples of aromatic amines which are unsatisfactory because of negative groups in the ring may be mentioned sulfanilic acid, anthranilic acid and o-chloro-m-toluidine-p-sulphonic acid.

65 The term "negative substituent" as used in this application has its usual meaning, namely, that it tends to increase the negative character or decrease the positive character of the molecule of which it is a part.

70 The unsubstituted aromatic amines, for example, aniline and the toluidines have not been found oxidizable under the conditions described.

75 It is sometimes desirable to add a wetting agent to the staining composition in order to obtain better penetration as for example sulfonated castor oil, one of the alkylated naphthalene sulfonic acids sold under the trade name of Nekal or tri-

5

10

15

20

25

30

35

40

45

50

55

ethanolamine oleate or other ethanolamine soap. Catalysts other than the cupric chloride of the examples are suitable. In general any soluble cupric salt, for example, cupric acetate may be used. The soluble salts of vanadium are suitable.

The invention is not limited to those solvents mentioned in the above examples, for example, benzene and acetone, give satisfactory results.

- 10 In general any organic solvent which may be classified as miscible or immiscible with water is suitable. Water itself may be used in cases where it is not harmful to the success of the process. The disadvantages of using water are
- 15 that it causes swelling of the wood and therefore requires considerable time for the wood to regain its normal dimensions in order that it may be further processed. Another objection to the use of water is present in the case where the wood
- 20 to be stained contains glued joints. The water loosens the joints.

In the case where the material to be stained is not swelled by water its use as a solvent is quite satisfactory especially with the more soluble compounds such as m-phenylene di-amine and the like.

- 25 All of the solvents covered by the above description may be generally divided into two classes known as polar, that is, one in which ionization takes place and non-polar, that is, one in which ionization is not appreciable, solvents. Where polar solvents are used the basicity of the amine or di-amine substance may cause precipitation of the catalyst and it is therefore necessary to add
- 30 to the solution a material which will cause retention of said catalyst in said solution. In Example II ammonia has been mentioned but this may be replaced by other compounds when their particular properties do not interfere with the process.
- 35 As examples of such compounds glycerine and tartaric acid may be cited.

While wood has been used for ease of description in the examples it is to be understood that the invention is broadly applicable to fibrous materials. Mention may be made of asbestos, wool, paper, paper pulp and fur.

The method of application may be varied widely in order to meet particular conditions. For instance in the process of Example III the order of application of the materials may be reversed. In other instances better and more rapid penetration may be secured by applying the stain producing compound under pressure. The penetration can be varied to the desired degree by the time of soaking. The method of drying may be modified as required by specific situations. The same generality applies to the concentration of the solutions used in the process and the temperature for the drying.

- 60 This invention has numerous advantages as will be obvious from a consideration of the specification. Because organic solvents are used wood articles comprising joints held together by water soluble glue may be stained satisfactorily. Furthermore, use of solvents of this character because of their high volatility results in quick drying of the material (30 minutes penetration of these compositions being equivalent to several hours penetration of the compositions heretofore known) and consequently permits rapid processing. Rapid processing is further aided by the fact that these solvents do not swell the wood being treated (as does water) and therefore the time required to allow an article to regain its normal size is eliminated. Because no

mineral acids are used in this invention tendering of the fibers of the materials stained is avoided. Because of the absence of chemical oxidizing agents in the process efflorescence on the stained article is not present. Another great advantage of the invention is that the stains produced are extremely fast and are not extracted by any ordinary method. Still another advantage is present in the fact that the grain of the wood stained according to this invention is 10 not obscured.

As many apparently widely different embodiments of this invention may be made without departing from the spirit and scope thereof, it is to be understood that we do not limit ourselves 15 to the specific embodiments thereof except as defined in the appended claims.

We claim:

1. The process of staining wood which comprises treating the wood with a composition of 20 matter comprising an organic solvent selected from the group consisting of alcohol, the mono-ethyl ether of ethylene glycol, benzene, acetone and toluene, a member selected from the group consisting of m-tolylene-diamine, m-phenylene- 25 diamine, p-phenylene-diamine, m-naphthylene-diamine, p-amino-phenol, and p-amino-anisole, and cupric chloride, and thereafter exposing the treated material to the action of air.

2. The process of staining wood which comprises treating the wood with a solution of cupric chloride in alcohol and aqua ammonia to which has been added m-tolylene-diamine, and thereafter exposing the treated material to the action 35 of air.

3. The process of staining wood which comprises treating the wood with a solution of m-tolylene-diamine in alcohol, subsequently treating the wood with a solution of cupric chloride in alcohol, and thereafter exposing the wood to 40 the action of air.

4. A composition of matter comprising an organic solvent selected from the group consisting of alcohol, the mono-ethyl-ether of ethylene glycol, benzene, acetone and toluene, a member selected from the groups consisting of m-tolylene-diamine, m-phenylene-diamine, p-phenylene-diamine, m-naphthylene-diamine, p-amino-phenol, and p-amino-anisole, and cupric chloride, the ingredients being in proportions which, on 45 exposure to air, impart a stain to wood impregnated therewith.

5. A composition of matter comprising a solution of cupric chloride in alcohol and aqua ammonia to which has been added m-tolylene-diamine, the ingredients being in proportions which, on exposure to air, impart a stain to wood 55 impregnated therewith.

6. The process of claim 1 in which the wood is first impregnated with the solution of the 60 amine and thereafter is impregnated with the solution of the catalyst.

7. The process of staining fibrous materials which comprises impregnating a fibrous material with one of a group of compounds consisting of 65 an aromatic mono-amine having a positive group substituted thereon and an aromatic diamine having a positive group substituted thereon in a solvent inert to the fibrous material, in another operation impregnating the fibrous material with 70 an oxidation catalyst in a solvent inert to the fibrous material, and exposing the treated material to the action of a gas containing free oxygen.